

June 7, 1949.

H. L. RATCHFORD

2,472,760

ELECTRODE FOR ELECTRON DISCHARGE DEVICES

Filed Dec. 30, 1943



HARRY L. RATCHFORD  
INVENTOR

BY *John J. Rogan*  
ATTORNEY

## UNITED STATES PATENT OFFICE

2,472,760

ELECTRODE FOR ELECTRON DISCHARGE  
DEVICESHarry L. Ratchford, Williamsport, Pa., assignor  
to Sylvania Electric Products Inc., Emporium,  
Pa., a corporation of Massachusetts

Application December 30, 1943, Serial No. 516,251

2 Claims. (Cl. 250—27.5)

1

This invention relates to electron discharge devices and more particularly to the electrodes used in discharge tubes operated at high temperatures.

One of the difficulties encountered in the operation of thermionic tubes operated or processed at high temperatures, as power and transmitting tubes, is the occurrence of uncontrolled electron emission from the control grid or any of the other "cold" discharge electrodes. It is in general desirable that the only source of electron emission be the thermionic cathode (the "hot" electrode), as primary and secondary electron emission from any of the cold tube electrodes influence the electrical tube characteristics in an undesirable manner.

In tubes designed for operation at high temperatures, the material of the grid electrodes must have a high melting point and must have high mechanical strength at high temperatures. These conditions are fulfilled for certain materials, e. g., tungsten, molybdenum, and tantalum. These materials do, however, have the undesirable feature that they have a tendency toward secondary and primary electron emission, and collect some of the emitter material evaporating from the thermionic cathode. Platinum, on the other hand, is very desirable as a material from the viewpoint of low secondary and primary electron emission. Unfortunately, the mechanical strength of platinum is comparatively low, in particular at high temperatures, and what is gained by the use of platinum as a grid material for high temperature operated tubes, considering its desirable low electron emission properties is lost again in view of the deficiency of this material in mechanical stiffness. The characteristics of tubes incorporating platinum grids vary widely from tube to tube, due to changes in the shapes of the grids made of this soft material during the processing or the life of the tube.

It is, therefore, a principal object of the invention to produce electron discharge tubes which can be processed and operated at high temperatures, and whose characteristics do not change from tube to tube of the same standard design as a result of the softness of their cold electrodes, and do not exhibit the undesirable effect typical of primary or secondary electron emission from these electrodes.

One object of the invention relates to means for increasing the mechanical stiffness of a grid made of platinum.

According to another object of the invention, means are provided to alloy the surface of a

2

platinum grid structure so as to increase its mechanical stiffness and to preserve the low electron emission properties of platinum.

Another principal object of the invention relates to the use of a platinum alloy as material for making grids for thermionic tubes operated at high temperatures, which incorporates the desirable low electron-emitting features of platinum combined with a mechanical stiffness considerably higher than that of platinum.

A feature of the invention relates to means for making grids which cannot be contaminated by the emitter material evaporating from the thermionic cathode during processing and life of the tube.

In the drawing there is shown in diagrammatic form a grid electrode embodying the invention.

The invention is based on the fact, that some of the physical properties of a metal are usually changed, while others remain constant when a pure metal is alloyed with one or several other metals. Recognizing the superior qualities of platinum as a grid material, with respect to its low electron-emitting properties, but recognizing also the deficiency of this material in mechanical stiffness, in particular at high temperatures, the present invention provides the possibility of alloying platinum with an appropriate "hardener," resulting in an alloy which will preserve the desirable low electron emission properties of platinum, but having the desirable increased mechanical stiffness.

According to one embodiment, there is provided an appropriate platinum alloy grid made from a grid made of pure platinum wire. For this purpose, the ready or preformed platinum grid is sprayed with a lacquer suspension of fine tungsten powder immediately preceding the mounting of the electrode assembly within the tube. The heat applied to the grid in the ordinary processing of the tube during exhaust running as high as 1600° C., results in the formation of a stiffer alloy, which however still preserves the low electron-emitting features of platinum. It was found that the grid emission of the tubes having platinum grids treated in this manner was substantially as low as that of tubes made with pure platinum grids. At the same time, the stiffness of the grids treated in this way was found to be considerably higher than that of the grids made of plain platinum wire, as demonstrated by comparative tests made with grids of both kinds, namely plain platinum grids and grids treated as described.

According to the above-described embodiment

of the invention, therefore, grids for use in tubes to be processed at high temperatures are made of platinum wire, then sprayed with a lacquer suspension of tungsten powder of approximately 325 mesh, then mounted into a tube in the conventional manner. The complete tube mounts are then processed as usual during the exhaust. As an example, a grid made of platinum wire of .012" diameter is sprayed with a suspension consisting of:

| Parts                                                             |
|-------------------------------------------------------------------|
| Medium viscosity nitro cellulose (approximately 20 seconds) ----- |
| Diethyl oxalate -----                                             |
| Butyl acetate -----                                               |
| Tungsten powder to 10 parts of above lacquer<br>(by weight) ----- |

mounted into a tube, which is then exhausted. During exhaust, the grid is heated to a temperature of 1500° to 1600° C., for five to ten minutes, whereby the desired alloying of the tungsten with the platinum takes place, resulting in increased stiffness of the grid structure and in substantial preservation of the low electron-emitting properties of pure platinum.

It will be understood that the invention is not limited to the particular method of alloying the tungsten and platinum described. Thus the platinum and tungsten may be alloyed in any well-known commercial manner and then drawn down to the wire size required for grid structures. Thus one alloy that was found suitable for the purpose above described contained approximately 2-6% tungsten and the balance platinum. Preferably, the tungsten should be 4% and the platinum 96%. Instead of using pure platinum with the tungsten a platinum rhodium alloy may be alloyed with the tungsten provided the platinum is the major part of the platinum rhodium portion of the alloy.

What is claimed is:

1. A wire grid electrode for use within an

electron tube and subjected to electron bombardment during the normal operation of the tube, said electrode comprising an alloy of approximately 96% platinum and 4% tungsten to increase the stiffness of the electrode while preserving the low electron-emissive properties of platinum.

2. A grid electrode for use in an electron tube of the type which employs a thermionic cathode tending to deposit emissive material on the grid during operation of the tube, said grid electrode comprising a platinum base alloy consisting mainly of platinum with from 2% to 6% tungsten for inhibiting primary emission from the grid when such emissive material is deposited thereon and for the purpose of increasing the stiffness of the electrode while preserving the low emissive properties of platinum.

HARRY L. RATCHFORD.

#### REFERENCES CITED

The following references are of record in the file of this patent:

#### UNITED STATES PATENTS

| Number    | Name       | Date          |
|-----------|------------|---------------|
| 803,684   | Fleming    | Nov. 7, 1905  |
| 1,096,655 | Weintraub  | May 12, 1914  |
| 1,236,383 | Fahrenwald | Aug. 7, 1917  |
| 1,342,801 | Gebauer    | June 8, 1920  |
| 1,346,192 | Gebauer    | July 13, 1920 |
| 1,407,525 | Fry        | Feb. 21, 1922 |
| 1,566,534 | Haagan     | Dec. 22, 1925 |
| 1,655,269 | Howe       | Jan. 3, 1928  |
| 1,719,774 | Metcalf    | July 2, 1929  |
| 2,032,694 | Gertler    | Mar. 3, 1936  |
| 2,183,635 | Barker     | Dec. 19, 1939 |
| 2,395,313 | Becker     | Feb. 19, 1946 |

#### FOREIGN PATENTS

| Number  | Country       | Date          |
|---------|---------------|---------------|
| 407,658 | Great Britain | June 14, 1932 |